

## UNITED STATES PATENT OFFICE

WILBUR B. DRIVER, OF EAST ORANGE, AND STANLEY R. KEITH, OF MONTCLAIR, NEW JERSEY, ASSIGNEES TO GILBY WIRE COMPANY, OF NEWARK, NEW JERSEY, A CORPORATION OF NEW JERSEY

## ELECTRICAL-RESISTANCE ALLOY

No Drawing.

Application filed July 3, 1930. Serial No. 465,643.

This invention relates to an alloy for electrical resistance uses.

For a long time the accepted alloy for resistance wires has been made from nickel-chromium. These two elements have given the highest electrical resistance for practical purposes when considered with their other properties. A resistance alloy must be capable of being worked, it cannot be brittle and must stand shocks and jars when in used. Iron is generally present in such alloys either as an impurity or because it is added to increase the workability of the alloy. A pure nickel-chromium wire has about 650 ohms C M F resistance. We have found that 65% Ni 15% Cr and 20% Fe produces the highest resistance that is 675 ohms.

One of the objects of this invention is to provide alloys of higher electrical resistance than nickel, chromium iron alloy.

Another object of this invention is to provide alloys of higher electrical resistance than nickel, chromium iron alloys that will have the proper properties to permit of workability, ductility and other properties to permit of use as resistance wire, strips, ribbon, sheet, castings, etc. A further object of this invention is to provide a series of alloys of the same elements having different electrical resistances of less than and greater than nickel-chromium-iron alloy.

If the alloy of nickel-chromium-iron is considered as a base and alloyed with manganese we have found that manganese up to 5% had practically no effect on the resistance but that from 10% on up the effect was positive and increased the resistance. Alloys much over 40% manganese proved brittle.

The following alloys have the following resistances:

| Ni % | Cr % | Mn % | Fe       | Resistance in ohms C M F |
|------|------|------|----------|--------------------------|
| 30   | 20   | 10   | Balance. | 635                      |
| 30   | 10   | 20   | Balance. | 650                      |
| 70   | 10   | 10   | Balance. | 650                      |
| 60   | 15   | 5    | Balance. | 675                      |
| 60   | 15   | 10   | Balance. | 710                      |
| 60   | 15   | 20   | Balance. | 785                      |
| 35   | 15   | 30   | Balance. | 845                      |
| 25   | 15   | 40   | Balance. | 795                      |
| 15   | 15   | 50   | Balance. | Brittle.                 |

If the alloy of nickel-chromium-iron is alloyed with vanadium we have found that vanadium also raises the resistance but unlike manganese its effect is great when but small amounts of vanadium are used as vanadium. 55 much in excess of 10% is too hard for workability.

The following alloys have the following resistances:

| Ni % | Cr % | Va % | Fe       | Resistance in ohms C M F |
|------|------|------|----------|--------------------------|
| 10   | 20   | 2½   | Balance. | 500                      |
| 10   | 10   | 3½   | Balance. | 550                      |
| 30   | 15   | 2½   | Balance. | 575                      |
| 40   | 10   | 2½   | Balance. | 615                      |
| 60   | 10   | 1    | Balance. | 650                      |
| 60   | 15   | 2½   | Balance. | 744                      |
| 75   | 15   | 2½   | Balance. | 790                      |
| 67   | 15   | 5    | Balance. | 790                      |
| 67   | 15   | 10   | Balance. | 810                      |
| 32   | 15   | 20   | Balance. | Too hard.                |

These alloys form satisfactory alloys with increased resistances.

It was found that manganese is equal to chromium in combination with nickel with respect to resistance while one part of the chromium is equal to two parts of manganese with respect to the hardening effect on the alloy's workability. We further found that when the ratio of nickel to chromium is less than 3:1 it is not workable.

We found that an alloy having the base of nickel, chromium and iron if alloyed with vanadium and manganese that resistances may be increased to almost double the resistance of the base and greater than with the use of either metal alone with the base.

For instance, the following alloys have the following resistances:

| Ni % | Cr % | Mn % | Va % | Fe       | Resistance in ohms C M F |
|------|------|------|------|----------|--------------------------|
| 35   | 15   | 30   | 2½   | Balance. | 932                      |
| 55   | 15   | 20   | 2½   | Balance. | 870                      |
| 45   | 15   | 30   | 2½   | Balance. | 934                      |
| 52   | 20   | 20   | 2½   | Balance. | 840                      |
| 43   | 10   | 40   | 2½   | Balance. | 1007                     |
| 50   | 5    | 40   | 2½   | Balance. | 1060                     |
| 48   | 10   | 30   | 5    | Balance. | 1073                     |
| 53   | 5    | 30   | 5    | Balance. | 1060                     |
| 38   | 10   | 40   | 5    | Balance. | 1070                     |
| 40   | 10   | 10   | 2½   | Balance. | 665                      |
| 40   | 10   | 20   | 2½   | Balance. | 760                      |
| 40   | 10   | 5    | 2½   | Balance. | 635                      |

From these alloys it can be seen that the alloys high in nickel and manganese show the greatest resistances.

When the ratio of nickel to chromium is less than three to one the alloy was too hard for workability, for instance:

35% Ni 15% Cr 40% Mn 2½% Va balance Fe resistance 1012 ohms C.M.F.  
25% Ni 15% Cr 30% Mn 5% Va balance Fe too hard.  
30% Ni 15% Cr 40% Mn 10% Va balance Fe too hard.

10 It will thus be seen that we have invented a series of resistance alloys whereby the base of nickel, chromium and iron is increased from 650 ohms to 1000 ohms by the addition of two elements which of themselves singly 15 do not materially increase the resistance but which in combination with the base do increase the resistances and which will have the proper properties for workability and use 20 for the purposes of electrical resistance material.

What we claim is:

1. An electrical resistance alloy, comprising vanadium 2.5%, manganese 40%, nickel 35%, chromium 15%, iron 7.5%.
- 25 2. An electrical resistance alloy comprising vanadium between 2% and 5%, manganese between 5% and 40%, nickel between 35% and 50%, chromium between 5% and 20%, and the balance iron.
- 30 Signed at Newark, in the county of Essex and State of New Jersey, this 11th day of June, A. D. 1930.

WILBUR B. DRIVER.  
STANLEY R. KEITH.

35

45

50

55

60

65